

## UNITED STATES PATENT OFFICE

HARALD SKAPPEL, OF OSLO, NORWAY

## PROCESS FOR SMELTING SULPHIDE ORES TO METAL, MATTE, AND SLAG

No Drawing. Application filed July 30, 1928, Serial No. 296,414, and in Norway October 15, 1928.

This invention relates to a process for smelting sulphide ores to metal, matte and slag.

In the existing metallurgical matte smelting in the lead, copper, and other non-ferrous metal industries, operations are carried on with the formation of slags rich in ferrous oxide (over 15% of FeO) and of mattes having a high power of dissolving pure metal.

10 In contrast thereto, the present process contemplates the formation of slags poor in FeO, and in equilibrium thereto, mattes which contain light-metal sulphides, thus facilitating a clean-cut separation between the crude 15 metal and the matte. The process is based on my newly discovered principles with regard to the stratification and distribution of the elements in the metallurgical polyphase system: metal, sulphide, silicate; employed in 20 combination with the old metallurgical smelting process.

If the various metallic sulphides be regarded, in a purely superficial manner, in the crystalline condition, it is found that some of 25 them, such as MoS<sub>2</sub>, PbS, NiS, CoS, Cu<sub>2</sub>S, and FeS, for example, have a typically metallic appearance, whilst others, such as SnS, CdS, and certain zinc blends etc., containing iron sulphide, are of semi-metallic aspect, 30 and others again, such as pure ZnS, MnS, etc., together with all the light-metal sulphides, have quite a non-metallic appearance. Closer investigation shows that the physical properties of the sulphides agree fairly well with 35 their appearance. For example, the "metallic" sulphides conduct the electric current in just the same way as metals, without undergoing transportation of substance; whereas the "non-metallic" sulphides, in the molten 40 state, conduct the electric current electrolytically (that is to say, with transportation of substance). A "metallic" property of certain heavy-metal sulphides, which is very important from the metallurgical point of view, 45 is their capacity for dissolving pure metal when they are in the molten state, and of being dissolved by pure metal. In the sulphide series, this property diminishes as the metallic nature of the sulphides in question becomes 50 less apparent. Thus, FeS, for example, is of

metallic appearance and, in the molten state and at a sufficiently high temperature, is miscible with metallic iron to an unlimited extent. On the other hand, Al<sub>2</sub>S<sub>3</sub>, for example, 55 has a non-metallic appearance, and is quite insoluble (in the molten state) in pure aluminium, or other pure metals. Pure metals, such as iron and aluminium, are mostly miscible to an unlimited extent in the molten state. If investigation be made into the fundamental 60 difference between a metal (M) and a sulphide (MS), formed out of its components in accordance with the equation M + S = MS + X (in which X represents the heat of formation), it is found, by comparing the various 65 sulphides, that the heat of formation plays an important part, in accordance with the law that "The metallic properties of the metallic sulphides decrease as the heat of formation per gram-atom of sulphur increases." In the 70 following table, the most usual metallic sulphides are arranged in the order of the increasing heat of formation per gram-atom of sulphur.

| Chem. formula                  | Heat of formation, cal. | Heat of formation pr. gram-atom of S, cal. | Nature and properties |    |
|--------------------------------|-------------------------|--------------------------------------------|-----------------------|----|
| Ag <sub>2</sub> S              | 3                       | 3                                          |                       | 80 |
| Hg <sub>2</sub> S              | 10.6                    | 10.6                                       |                       |    |
| As <sub>2</sub> S <sub>3</sub> | (?)                     | (?)                                        |                       |    |
| Sb <sub>2</sub> S <sub>3</sub> | 34.4                    | 11.5                                       |                       |    |
| MoS <sub>2</sub>               | (?)                     | (?)                                        |                       |    |
| NiS                            | 19.3                    | 19.3                                       |                       |    |
| PbS                            | 20.2                    | 20.2                                       |                       |    |
| Cu <sub>2</sub> S              | 20.3                    | 20.3                                       |                       |    |
| CoS                            | 21.0                    | 21.9                                       |                       |    |
| FeS (crystalline)              | 24                      | 24                                         |                       |    |
| FeS (amorphous)                | 18.8                    | 18.8                                       |                       |    |
| SnS                            | (?)                     | (?)                                        |                       |    |
| Cr <sub>2</sub> S <sub>3</sub> | (?)                     | (?)                                        |                       |    |
| CdS                            | 34.4                    | 34.4                                       | Semimetallic.         | 85 |
| Al <sub>2</sub> S <sub>3</sub> | 126.4                   | 42.1                                       |                       |    |
| ZnS                            | 43                      | 43                                         |                       |    |
| MnS                            | 45.6                    | 45.6                                       |                       |    |
| MgS                            | 79.4                    | 79.4                                       |                       |    |
| Na <sub>2</sub> S              | 89.3                    | 89.3                                       |                       |    |
| CaS                            | 94.3                    | 94.3                                       |                       |    |
| SrS                            | 98.3                    | 99.3                                       |                       |    |
| BaS                            | 102.9                   | 102.9                                      |                       |    |
| K <sub>2</sub> S               | 103.5                   | 103.5                                      |                       |    |
| Li <sub>2</sub> S              | 105                     | 105                                        |                       |    |

It appears that metallic sulphides with less than about 28 cal. per gram-atom of sulphur possess "metallic" properties, whereas metallic sulphides with a heat of formation exceeding 40 cal. per gram-atom of sulphur 100

are decidedly "non-metallic". The table shows further that the "metallic" sulphides consist exclusively of those of the heavy metals, whereas all the light-metal sulphides and only the sulphides of the most active heavy metals (such as Zn, Mn) are "non-metallic". The term "light metals" in the specification and claims is intended to include the alkali and alkaline earth metals and all metals whose atomic weight does not exceed 40.07. The further peculiarity exists that, with few exceptions, all the sulphides are mutually soluble in the molten state; and moreover, that the metallic character of such solutions of one sulphide in another depends in such a manner on the mean heat of formation per gram-atom of sulphur, that mixed sulphide melts with a mean heat of formation of less than about 24 cal. per gram-atom of S are "metallic" whilst mixed sulphide melts with a mean heat of formation exceeding about 40 cal. per gram-atom of sulphur are "non-metallic". (The numerical values of the mean heat of formation to be maintained for the mixed sulphides melts relate, here and hereinafter, always to a heat of formation, of FeS, of 24 cal. per gram-atom of S.) This discovery affords a means of controlling the stratification in the metallurgical polyphase system: metal, sulphide, silicate. The present metallurgical practice is to operate with decidedly "metallic" sulphide melts (or "mattes"), which possess a high solvent power for pure metals, so that fractionated separation of crude metal from said mattes in the molten state can only be effected in a very imperfect manner. If however, in accordance with the principle enunciated above, there be added to such mattes so much sulphide with a higher heat of formation that the mean heat of formation of the sulphide melt increases to about 25-35 cal. or more per gram-atom of S, then the matte loses its property of holding pure metal in solution. The pure metal which was held in solution is transferred to a metallic phase which is sharply divided from the sulphide phase, even in the melt. For practical success with the process, it has been found advantageous to keep the sulphide phase covered with a silicate slag. The stratification of metal and sulphide occurs very quickly and finely if care be taken, by a short thermo-electrolytic treatment,—in which the silicate phase is connected up as the electrolyte, and the sulphide and metal as the cathode—to ensure the rapid attainment of chemical equilibrium between the phases. With a sulphide layer containing light-metal sulphides, however, this state of equilibrium can also be attained in the first stage of smelting, by selecting a suitable composition for the charge and a suitable amount of added reducing carbon; and such method of smelting, with the results accruing there-

from, is the actual subject of the present invention.

A point of importance to the regulation of the stratification and the cleanliness of the separation of the strata in the metallurgical polyphase system: metal, sulphide, silicate, is the inventor's discovery that, not only is the sharpness of the separation between metal and sulphide dependent on the decrease of energy between these phases, but, in addition, the separation between sulphide and oxide, or silicate, is dependent on the decrease of energy between the phases. If therefore, a clean separation between sulphide and metal is effected by the addition of a light-metal sulphide, the decrease of energy between sulphide and silicate is lessened at the same time, thereby increasing the mutual solubility of these phases. For this reason, the addition of light-metal sulphide must not be carried too far in operating with the three-phase system. It has been found of advantage in practice to maintain the mean heat of formation of the sulphide stratum between 25 and 35 cal., per gram-atom of S.

A point of importance for estimating the decrease of energy between sulphide and oxide is my discovery that, in the oxide series also—though not in such a notable degree as in the sulphides—there are members of a "metallic", "semi-metallic" and "non-metallic" character; but that the absolute values of the heat of formation of corresponding sulphides and oxides differ considerably, inasmuch as the "metallic" character of the metallic oxides evidently extends over a wider energy interval than is the case with the sulphides. It is well known that cuprous oxide is highly soluble in molten copper, although the heat of formation of cuprous oxide is 43.8 cal., at which level the sulphides, such as ZnS, MnS and  $Al_2S_3$  are completely non-metallic. The iron-oxide ores with heats of formation of about 65 cal. per gram-atom of oxygen, have a "metallic" and "semi-metallic" appearance. The boundary between "semi-metallic" and "non-metallic", which in the case of the sulphides lies between 39 and 40 calories per gram-atom of sulphur, appears, in the case of the oxides, to lie between 70 and 80 cal. per gram-atom of oxygen. Zinc oxide, with a heat of formation of 84.8 cal. is pure white and non-metallic; and its position in the oxide series probably corresponds approximately to that of zinc sulphide (43 cal.) in the sulphide series. At an energy interval of about 80 cal. per gram-atom of oxygen between metal and metallic oxide, the solubility of the oxide in the metal has practically ceased to exist. Hence, in a manner analogous to that observed with the sulphides, a clean separation in relation to the metal phase (or sulphide phase) can also be effected in this case by sufficiently increas-

ing the energy interval between the phases by the addition of oxides with a higher heat of formation. In selecting the added oxides, care must be taken to ensure that they possess sufficient affinity towards the oxides with lower heat of formation present.

As has been ascertained by the inventor, the aforesaid conditions for a sharp demarcation, both between metal and sulphide, and also between sulphide and silicate (or oxide), can be fulfilled in a single smelting operation, by maintaining definite charging conditions in smelting. The apparatus and performance of the operation remain substantially as at present customary, but the entire course of the smelting is performed, so to speak, in a different range of the metallurgical polyphase system: metal, sulphide, slag, inasmuch as the "degree of reduction" (hereinafter more fully defined) of the system is substantially increased. In order to understand the relative conditions in this connection, and to operate accordingly, it is necessary to be well informed with regard to the various states of chemical equilibrium of the metallurgical polyphase system: metal, sulphide, silicate under different conditions as to the content of oxygen and sulphur.

The chemical equilibrium of the system: metal, sulphide, silicate, may be regarded as the result of a contest of all the elements present for insufficient quantities of sulphur and oxygen. In these circumstances, the elements distribute themselves among the various phases in such a manner that the free energy of formation of the whole system attains a maximum. As has been ascertained, the stratification of the system in the melt is also dependent on the energy of formation of the various liquid phases, inasmuch as certain decreases of energy occur, both from metal to sulphide and from sulphide to oxide or silicate, these decreases forming the chief cause of the separation of the phases.

If sulphur be added to the system, then an equivalent amount of metal is transferred, accompanied by the evolution of energy, from the metal phase to the sulphide phase. If oxygen be added to the system, then an equivalent amount of metal is transferred, accompanied by the evolution of energy, from the metal phase into the sulphide phase, and at the same time the corresponding amount of metal is transferred from the sulphide phase into the silicate phase. If, on the other hand, oxygen be withdrawn from the silicate phase, by the addition of energy, the equivalent amount of metal will be transferred from the silicate phase into the sulphide phase, and at the same time the equivalent amount of (other) metal will be given up by the sulphide phase to the metal phase. At the same time, both the transference of elements from

the silicate phase to the sulphide phase, and the simultaneous cession of metal from the sulphide phase to the metal phase, take place in a certain serial order, inasmuch as the elements whose transference requires the smallest addition of energy to the system are the first to be transferred. Usually, however, several elements are transferred simultaneously, but in different relative proportions, according to their concentration in the phases and their position in the serial order of transference from silicate to sulphide, or from sulphide to metal.

The inventor has previously described in his application Serial No. 694,609 a process which enables the amount of oxygen or sulphur in the molten system: metal, sulphide, silicate, to be gradually lowered, so that the entire chemical equilibrium of the system is displaced. The experimental performance of the process has therefore afforded an excellent opportunity of investigating the various states of equilibrium of the metallurgical polyphase system at various degrees of reduction. The process consists in employing the silicate phase (or slag) as electrolyte. The metal phase and sulphide phase are connected up as cathode, whilst a carbon electrode dipping into the silicate phase is employed as anode. When the current is switched on, the cations of the silicate phase migrate towards the surface of the cathode sulphide phase, and are there transferred, in a certain serial order, from silicate or oxide into sulphide, an equivalent amount of metal being ceded from the sulphide phase to the metal phase at the same time. The anions (chiefly  $\text{SiO}_3$ ) of the silicate phase migrate at the same time towards the carbon anode, where they are neutralized, by giving up oxygen which combines with the anode material and escapes as carbon monoxide. So long as the electrolysis takes this course, it can be typically represented by the following reactions:



If these reactions be established for the most important elements occurring in the silicate phase (or slag)—for example, for the decomposition of  $\text{FeS}$ —the differences in the heat effects per gram-atom of S furnish a survey of the serial order in which the various components of the silicate phase are transferred. In all these reactions, CO is liberated at the anode, and Fe is separated cathodically so that the difference in the energy required for transforming the elements from silicate, or oxide, into sulphide, may be expressed by the differences of the heat effects per gram-atom of S, and those components which require the smallest amount of energy for the conversion

are naturally converted first. The reactions such a way that one element is transferred are set out in the appended Table 2:

TABLE 2

|    |                                                        | Cal.        | Per 1 gram-atom of S kg.-cal. | 70 |
|----|--------------------------------------------------------|-------------|-------------------------------|----|
| 5  |                                                        |             |                               |    |
| 1  | $FeS + K_2O + C = Fe + K_2S + CO$                      | + 10.4      | + 10.4                        |    |
| 2  | $FeS + Na_2O + C = Fe + Na_2S + CO$                    | + 2.5       | + 2.5                         |    |
| 3  | $FeS + BaO + C = Fe + BaS + CO$                        | - 25.4      | - 25.4                        |    |
| 4  | $FeS + Li_2O + C = Fe + Li_2S + CO$                    | - 29.8      | - 29.8                        |    |
| 5  | $FeS + CaO + C = Fe + CaS + CO$                        | - 32.1      | - 32.1                        |    |
| 6  | $FeS + FeO + C = Fe + FeS + CO$                        | - 36.5      | - 36.5                        |    |
| 7  | $FeS + ZnO + C = Fe + ZnS + CO$                        | - 36.6      | - 36.6                        |    |
| 8  | $FeS + MnO + C = Fe + MnS + CO$                        | - 40.1      | - 40.1                        |    |
| 9  | $FeS + MgO + C = Fe + MgS + CO$                        | - 58.9      | - 58.9                        |    |
| 10 | $3FeS + Al_2O_3 + 3C = 3Fe + Al_2S_3 + 3CO$            | - 250.7     | - 83.6                        | 75 |
| 11 | $3FeS + B_2O_3 + 3C = 3Fe + B_2S_3 + 3CO$              | - 181.3     | - 60.4                        |    |
| 12 | $2FeS + SiO_2 + 2C = 2Fe + SiS_2 + 2CO$                | - 129.8     | - 44.8                        |    |
| 13 | $2FeS + TiO_2 + 2C = 2Fe + TiS_2 + 2CO$                | - (?)       | high                          | 80 |
| 14 | $FeS + ZnSiO_3 + C = Fe + ZnS + SiO_2 + CO$            | - 39.5      | - 39.5                        |    |
| 15 | $FeS + BaSiO_3 + C = Fe + BaS + SiO_2 + CO$            | - 40.0      | - 40.0                        |    |
| 16 | $FeS + Na_2SiO_3 + C = Fe + Na_2S + SiO_2 + CO$        | - 41.6      | - 41.6                        |    |
| 17 | $FeS + FeSiO_3 + C = Fe + FeS + SiO_2 + CO$            | - 45.4      | - 45.4                        |    |
| 18 | $FeS + MnSiO_3 + C = Fe + MnS + SiO_2 + CO$            | - 45.5      | - 45.5                        |    |
| 19 | $FeS + CaSiO_3 + C = Fe + CaS + SiO_2 + CO$            | - 49.0      | - 49.0                        |    |
| 20 | $FeS + MgSiO_3 + C = Fe + MgS + SiO_2 + CO$            | - (?) about | - 71.0                        | 90 |
| 21 | $4FeS + Al_2SiO_5 + 3C = 4Fe + 2SiS_2 + Al_2O_3 + 4CO$ | - 274.3     | - 68.6                        | 85 |
| 22 | $3FeS + Al_2SiO_5 + 3C = 3Fe + Al_2S_3 + 2SiO_2 + 3CO$ | - 265.6     | - 88.5                        |    |
| 23 | $FeS + Li_2SiO_5 + C = Fe + Li_2S + SiO_2 + CO$        | - 94.8      | - 94.8                        |    |
| 24 | $2FeS + Li_2SiO_5 + 2C = 2Fe + SiS_2 + Li_2O + 2CO$    | - 194.8     | - 97.4                        |    |

The reactions 1-10 furnish an idea of the conditions arising when the oxide phase, or silicate phase, is highly basic; whereas the reactions 11-24 correspond to the conditions with neutral or acid silicate phase. The difference between basic and acid slags is particularly small in the case of aluminium (reactions 10 and 22) and particularly great in the case of lithium (reactions 4 and 23). From the heat effects of the reactions 14-18 it is evident that the metals zinc, barium and sodium are situated, in the serial order of transference, from silicate to sulphide, closely in front of the position of iron, whilst manganese, on the other hand is beyond, whereas calcium and magnesium require more—and aluminium very much more—energy for their transformation from silicate into sulphide. In connection with the present process, it is highly interesting to note that the position of the light metals potassium, sodium and barium in the serial order of transference from silicate to sulphide is before or near to that of iron, that is they are converted from silicates to sulphides with a smaller consumption of energy than iron, thereby affording a means of smelting a matte containing light-metal sulphides, which is in equilibrium with the slag, even in cases where the slag contains relatively large amounts of ferrous oxide. To do this, all that is needed is to add sufficient amounts of the said light metals to the system.

Practical tests confirm the serial order of transference from silicate to sulphide indicated by the table, which is approximately as follows:

60 Nobler heavy metals (for example Pt, Au, Ag, As, Sb, Mo, Ni, Co, Cu, Pb)—Zn, (Sn), —K, —Na, —Ba, —Fe, —(Cr), —Mn, —Ca, —Mg, —Al, —(Li).

65 Of course, in carrying out the process in practice, this serial order does not occur in

differentiation from the latter, but the matter is one of a displaceable chemical equilibrium—adjustable within small intervals—in which the distribution of the elements present, in silicate, sulphide and metal is determined, and by the degree of reduction fixed for the time being. From this it is clear that the degree of reduction is determined by the last element transferred into the sulphide phase; so that, in theory, there are as many degrees of reduction as there are elements in the transference series. This simple fact was previously unknown in metallurgy; and its discovery enables the metallurgical polyphase system to be dealt with in quite a different manner from heretofore, inasmuch as it is possible by maintaining certain degrees of reduction to drive over certain elements completely, for example into the sulphide phase, if their position in the transference series be known, or determined by preliminary experiment.

If, for example, a molten mixture of oxides, or a silicate phase, be added to molten iron sulphide—such addition containing a sufficient amount of oxides of other of the nobler heavy metals, in addition to the usual slag constituents—then, as is known from the older metallurgy, the major portion of the heavy metals nobler than iron, will be transferred from the silicate phase to the sulphide phase, by a purely chemical reaction (expressed by the equation  $Cu_2O + FeS = Cu_2S + FeO$ ) between the silicate phase and the sulphide phase, inasmuch as they are replaced in the silicate phase by the equivalent amount of iron. In this manner, a silicate phase is obtained of approximately the same composition as the ordinary slags of matte smelting, which are rich in ferrous oxide. In this case, the FeS content of the sulphide phases forms, as it were, a guarantee against the slagging of

the nobler heavy metals. Only such heavy metals as occupy a position near that of iron in the series of transference from silicate to sulphide—for example, zinc, manganese, chromium, etc.—will remain—like the iron—in any considerable quantity in the silicate phase. If this silicate phase be still further reduced, for example by the previously mentioned thermo-electrolysis, transfer from silicate to sulphide will be chiefly effected in the case of iron, at the commencement of the electrolysis, accompanied, however, in certain relative proportions, by the said heavy metals, Zn, Mn, etc., and also by light metals such as potassium, sodium and barium, which can be transformed from oxide into sulphide just as easily as iron. At the same time, the already low content of nobler heavy metals in the silicate phase will be still further lowered. Not until the reduction has proceeded so far that the content in the silicate phase of  $(FeO + FeS)$ —has been reduced to a certain extent—to about 7%  $(FeO + FeS)$  in basic slags, and considerably less in acid slags—do any notable amounts of calcium and magnesium begin to be transformed into sulphide. At the same time, FeS ceases to act as a preventive of the slagging of nobler heavy metals, this role being assumed by the content of calcium sulphide and magnesium sulphide in the sulphide phase. As reduction progresses, especially when the amounts of calcium oxide and magnesium oxide in the silicate phase have become very small, the more difficultly transferable oxides, such as aluminium oxide, begin to pass over into sulphide in notable amount. By carrying the reduction further, the entire oxide, or silicate phase may, in certain circumstances, be completely eliminated.

It follows therefore that the distribution of the various elements in the three-phase system: metal, sulphide, silicate, varies with the above defined degree of reduction of the system, and, in respect of the relation between slag and matte, and with reference to the components usually present in the slags and mattes, the entire system may be suitably grouped into the following stages of reduction:

1. The ferrous oxide stage, which is characterized by a silicate phase rich in FeO—down to about 7% FeO—and by a sulphide phase which is almost free from CaS, MgS,  $Al_2S_3$ , etc., but mostly rich in FeS, inasmuch as, in this stage, the iron sulphide forms the protection against the oxide slagging of the nobler heavy metals. If the silicate phase be acid, the limit of the stage is reached with far smaller contents of ferrous oxide than specified above. In this stage, a considerable percentage of the baser heavy metals, such as Zn, Sn, Cr, Mn, etc., is taken up, or slagged, by the silicate phase, together with ferrous oxide; whereas certain light metals, such as K,

Na and Ba, are already partly transferred into the sulphide phase during this stage. The loss of nobler heavy metals, such as Pb and Cu, by slagging, is sensible in this stage, especially when operating with a high FeO content.

2. The calcium sulphide stage is characterized by a light-metal silicate phase—low in iron and containing CaO and/or MgO—and a heavy-metal sulphide phase containing CaS and/or MgS. In this stage, the baser heavy metals, Zn, Cr, Mn, Fe, etc., are also fairly extensively transformed into sulphide, together with the light metals K, Na, Ba, etc., to an increased extent. In this stage, CaS and MgS form the protection against oxide slagging of the nobler heavy metals, which is considerably lessened by comparison with the first stage.

3. The aluminium sulphide stage, characterized by a silicate phase or oxide phase which is low in FeO, CaO and MgO, and is constituted by the light-metal oxides or silicates (such as  $Al_2O_3$ , etc.) which are most difficult to transform into sulphide, and of a heavy-metal sulphide phase containing  $Al_2S_3$ , if any heavy-metal sulphide be present. Light metal oxides of K, Na, Ba, Ca, Mg, etc., can be transformed into sulphides in this stage almost completely. Silicon, aluminium and lithium can also be extensively transformed into sulphide or to the elementary condition, in this stage.

These groups, or stages, which broadly indicate the serial order of transformation of silicate into sulphide, can, of course, be further sub-divided as desired, inasmuch—as already mentioned—as there exists, for each constituent of the silicate phase, a certain (adjustable) degree of reduction of the system, at which it is transformed into sulphide in a practically complete manner. Regarded from this standpoint the hitherto known metallurgical treatment of the non-ferrous metals is uneconomical insofar as on an average, slags, which are very rich in ferrous oxide, (containing from 18 up to over 50% FeO) are employed, that is to say, slags of an extremely low degree of reduction and thus a correspondingly high oxidic slagging both of the more noble metals (such as for example, Ag, Cu, Ni, Co, Pb), and particularly of the baser heavy metals (such as for example, Zn, Sn, Cr, Mn, etc.).

In contradistinction to this, the present invention contemplates altering the course of the melting in the smelting of for example, copper ores, lead ores, lead-, zinc-, copper-ores, copper-, zinc-, silver ores, complex tin ores and others in such a manner that a system of a very high degree of reduction—more closely defined as slagging—is employed, which contains from 15% to 0% FeO and mattes containing from 1.5 to 20% and in certain cases less than 1.5% and more than

20% of light metal sulphide (taking into consideration the average heat of formation hereinbefore set forth). Whereas the present day metallurgy removes manganese, zinc and other base heavy metals from such mixtures of ore by slagging, the present invention aims at collecting them mainly in the mattes. This is attained not only by the higher degree of reduction but also by the fact that wherever possible, extremely acid slags are employed insofar as it is known that, as the acidity of the slags increases their solvent properties for sulphide decrease. By increasing the degree of reduction a more complete transformation of the desired constituents into sulphide is thus obtained and by increasing the acidity of the slag the result is obtained that the (metallic or non-metallic) sulphides formed substantially collect in the matte. If it be assumed that slags of these three stages are in contact with mattes of one and the same composition, then the decrease in energy hereinbefore referred to between silicate phase and sulphide phase in the ferrous oxide stage is at a minimum, and is greater in the calcium sulphide stage and at its maximum in the aluminium sulphide stage and the greater the decrease in energy the more complete is the separation of the phases.

In cases where only the two phase: sulphide, silicate, system is being worked up the same considerations arise as in the three phase: metal, sulphide, silicate system. However also where the sulphide phase is absent, that is to say, in the metal, silicate, system, similar considerations must be taken into account and there is a transformation series of the elements from silicate or oxide to metal. In a few individual cases, this occurs in metallurgy without the principles in question however, being clearly recognized. The best proof of this, is the existing practice in the metallurgy of tin ores, where on an average slags rich in ferrous oxide (18 to 50% Fe) were employed and as a consequence slags were produced even after twice smelting, which contain not less than 2 to 3% of tin. In the metallurgy of tin the recognition is obviously lacking, that the tin in the series of transformation from silicate or oxide to metal is so closely in front of the position of iron that a complete de-tinning of the slags can only take place with the simultaneous lowering of the ferrous oxide content of the slags. By increasing the degree of reduction of the tin slags it is easily possible, according to the present process to produce waste slags containing far less than 1% of tin.

Since one of the most important functions of the ferrous oxide content of the present matte slags is that of serving as a flux for lowering the melting point of the slags it is necessary in the present new process to

produce a melting point-lowering substitute for FeO. Such melting point-lowering agents may be alkalis, particularly Na<sub>2</sub>O, which can be added in the form of any cheap salt. A content of 3 to 10% alkali in the melt is usually sufficient for this purpose. Similarly, in order to lower the melting point of the mattes when they have a high content of difficultly fusible sulphide, such as for example ZnS, MnS, MoS<sub>2</sub>, it is possible to use in addition to other sulphides, alkali sulphide which at the same time produces the desired reduction of the dissolving power of the mattes for pure metal. By virtue of the composition of the charge and the degree of reduction of the system determined thereby, the result is attained that the added alkali salt etc., is divided up into desired portions between slag and matte. It has been shown that the addition of alkali has an extremely favourable effect on the course of the reactions insofar as it acts, so to speak, as a lubricant, so that the reactions take place at considerably lower temperatures than otherwise. The action of the added alkali is particularly noticeable when reactions analogous to those set forth in Table No. 2 are to follow a purely thermal course. The particularly important reactions:—



take place only at very high temperature because the reacting substances and the products of reaction (CaS and MgS) are very difficult to fuse. In consequence of the very high temperatures required these reactions which were hitherto known only strictly in a metallurgical sense for the desulphurization of iron, are of little use in the metallurgy of the non-ferrous metals. In the presence of a certain amount of alkali they take place smoothly and with ease at 1100 to 1400° C. By virtue of this, these reactions acquire a new utility and they open up new fields of use. A particularly novel and important application lies in the employment of the reactions in order to separate out fractionally one or more metals according to the present process, as crude metal from unroasted sulphide ores. For this purpose it is possible to supply with advantage as an example of material containing CaO and MgO, basic blast furnace slags or slags obtained in the production of steel, and alkali, for example, in the form of a suitable mixture



About 10% Na<sub>2</sub>SO<sub>4</sub> of the weight of the slag is sufficient. The slag is advantageously comminuted and mixed with the ore which is likewise comminuted and if desired preliminarily treated to bring same to the lowest possible stage of sulphurization, and is also

mixed with coke and sulphate and the mixture is, if desired, agglomerated (or briquetted), by moistening and drying the same prior to smelting. The smelting can be carried out in known manner and particularly in shaft furnaces or electric furnaces. Since larger amounts of CaS or MgS render both mattes and slags difficultly fusible, it is possible, in accordance with the principles here-

10 *inafter explained, by the simultaneous addition of old matte slags, rich in ferrous oxide and in the form of pieces, to provide for transforming CaS and MgS into CaO and MgO, which pass into the slag, (see for example, Example No. 1 below).*

From the foregoing explanation, numerous practical conclusions can be drawn. If, for example matte slags rich in ferrous oxide are smelted together with material yielding 20 CaS or MgS, for example CaS, anhydrite or gypsum and carbon, lime and material yielding sulphur, magnesium sulphate and carbon and the like, the transformation takes place during the melting down whereby the bulk 25 of the iron content of the matte slag is transformed into sulphide and forms matte in accordance with reactions analogous to the equations:—



30 inasmuch as the said matte is replaced by CaO or MgO in the slag. The operation represents on the one hand a process for utilizing the sulphur content of calcium sulphide, gypsum, anhydrite, etc., this being found to combine with iron or other heavy metals in which form it can be rendered useful in known manner by roasting, and on the other hand a process for the extraction of 40 iron and other heavy metals from silicates or slags inasmuch as these heavy metals are also transformed into sulphur compounds adapted to be more easily worked up. Simultaneously the slag is converted from ferrous 45 silicate into the more valuable calcium or magnesium silicate which on suitable adjustment of the composition either directly or by subsequent treatment (in the fused state), can be withdrawn as a valuable product for 50 example for cement, glass, brick, raw material for the manufacture of alumina etc.

In the direct smelting of sulphide ores rich in sulphur to form matte and slag, the distillable sulphur can be absorbed by the mixture of lime or limestone for example according to the equations:—



60 and the freshly formed CaS can be caused to react with old matte slags and to transform them into calcium silicate low in FeO whilst extracting the content of iron and heavy 65 metal in the form of sulphides. This re-

action can also be utilized for the purpose of slurring the CaO— and MgO— content of basic ores, by means of old matte slags rich in ferrous oxide, by first transforming <sup>70</sup> CaCO<sub>3</sub> and MgCO<sub>3</sub> of the basic ores into sulphides by the addition of pyrites or pyritic ores and carbon to the said ores and heating the mixture, the calcium or magnesium sulphides then reacting with the slags rich in ferrous oxide.

75 A particularly important field of application of the double decomposition between CaS and MgS and ferrous silicate is the direct working up in the fused state, of the slag derived from the smelting of matte, rich in ferrous oxide as obtained from the present smelting processes, into silicate with a low ferrous oxide content and a fresh matte which retains practically the whole of the content of the more valuable heavy metals <sup>80</sup> such as Cu, Pb, Ag, Sn, Zn, etc., remaining in these slags. The operation is preferably carried out in a fore hearth which is heated electrically or by other means and the operation of mixing CaS, MgS and if desired, <sup>85</sup> alkali sulphide with the slag is facilitated by the further addition of FeS or comminuted poor matte (if desired of the same operation) which produces a sinking of the light metal sulphide in the melt. The slag is according- <sup>90</sup> ly so to speak, treated by a double matte and is therefore extracted to a very great degree. By maintaining a definitely high degree of reduction, (for example by means of MgS) <sup>95</sup> it is possible in the second matte, under certain conditions, to cause the valuable rare elements present in the first slag such as for example, vanadium, tungsten, gallium, etc., to be deliberately driven over into the matte.

100 *Example No. 1*—A complex ore showed <sup>105</sup> on analysis, the following composition: 35.4% Pb, 9.4% Cu, 11.7% Zn, 4.9% Fe, 0.9% As, 17.1% S, 16.3% SiO<sub>2</sub>, 1.2% Al<sub>2</sub>O<sub>3</sub>, 1.1% CaO, 1.7% MgO. The ore was comminuted and mixed with 10% of quick lime, 10% <sup>110</sup> Na<sub>2</sub>SO<sub>4</sub> and 6% of powdered coke, agglomerated by moistening and drying and was melted in a shaft furnace, with the further addition of 20% slag rich in ferrous oxide, in known manner by means of coke in the form of pieces. An acid slag poor in ferrous oxide and having a very low content of heavy metal was obtained, together with the following products which could be separated by tapping <sup>115</sup> from each other:

1. Matte, of the composition: 8.3% Pb, 20% Cu, 23% Zn, 10.7% Fe, 0.49% As, 80 grams per ton of Ag, 9.7% (Na<sub>2</sub> + CaS) as well as S.

2. Speiss of the composition: Fe 68.3%, As 24.7%, Cu 3.2%, Pb not determined.

3. Workable lead with 580 grams per ton of Ag and only 0.56% As. It is remarkable <sup>125</sup> that in consequence of the content of light

130 metal in the matte, the lead is workable.

metal sulphide in the matte, in this method of carrying out the smelting, matte and speiss can be separated in a fluid state by tapping off from the fore-hearth.

- 5 *Example No. 2.*—A foundry had available a calcareous zinc ore of approximately the following composition: 9.6% Zn, 8.4% Fe, 3.5% Pb, 9.8% S, 2.6% SiO<sub>2</sub>, 66% CaCO<sub>3</sub> which was of such a nature that it could only be dressed 10 with great difficulty. The same works had at their disposal from a lead shaft furnace operation, unlimited amounts of old slags of the composition: 37.5%, SiO<sub>2</sub>, 28.4% FeO, 7.8% Al<sub>2</sub>O<sub>3</sub>, 14.7% CaO, 3.6% MgO, 6.2% 15 ZnO, 0.7% PbO, 0.4% Cu. During the treatment of these products according to the present process, it was attempted to collect the zinc content of the ore and the slag in a matte whereas the lime content of the ore was intended 20 to be converted into CaS by heating with the addition of imported iron pyrites of the approximate composition: 75% FeS<sub>2</sub>, 6% ZnS, 2% CuS, 1% PbS and 16% SiO<sub>2</sub>, in order subsequently to cause it to react with 25 the FeO content of the slag. In order to reduce the melting point of the matte it was treated so as to contain Na<sub>2</sub>S by the further addition of sodium sulphate and carbon whilst simultaneously the melting point of the slag 30 was reduced by taking up Na<sub>2</sub>O and it was prepared for conversion into bottle glass. Accordingly 1 ton of ore in a comminuted state was mixed with 1.5 tons of iron pyrites, 150 kgs. of sodium sulphate and 130 kgs. of coke powder and was agglomerated by moistening with water and subsequently drying. The whole was then fused in a shaft furnace together with 1.5 tons of old slag and coke, and about 1.87 tons of matte having the composition: 73% FeS, 17.3% ZnS, 3.7% PbS, 2.7% Cu<sub>2</sub>S, 2.5% Na<sub>2</sub>S, and 0.5% CaS, were obtained. This matte was worked up in known manner by crystallization, disintegration and dressing into zinc blend, magnetic 45 pyrites and copper-, lead-, silver-, sulphide-concentrate and in addition about 1.65 tons of slag having the composition 48.7% SiO<sub>2</sub>, 7% Al<sub>2</sub>O<sub>3</sub>, 35.1% CaO, 3.2% MgO, 3% FeO, 1.2% Na<sub>2</sub>O, 1.2% ZnS, 0.16% PbS and 0.18% 50 Cu<sub>2</sub>S, were produced. Such a slag can be worked up in another furnace into bottle glass, building brick or the like, after suitable adjustment of its composition.
- 55 *Example 3.*—A tin slag from a reverberatory furnace smelting operation contained: 39.4% SiO<sub>2</sub>, 14.7% Al<sub>2</sub>O<sub>3</sub>, 26.2% FeO, 7.9% CaO, 0.5% MgO, 1.7% Na<sub>2</sub>O, 8.1% SnO, 1.3% WO<sub>3</sub>. It was smelted together with a mixture of gypsum, sodium sulphate and carbon in suitable proportions. In this operation the tin, tungsten and iron contents of the slag were transferred to a matte containing sodium sulphide which was worked up in known manner into tin, tungsten and iron sulphide.

A further very important application of the process consists in working up certain oxidic ores into sulphides and slags with the aid of material which yields CaS or MgS and in particular ores which contain such 70 oxides of heavy metals which lie in the vicinity of iron or after iron in the serial order of transference from oxide to sulphide, such as for example, the chromium and iron content of chrome-iron-stone, the manganese 75 content of impure manganese ore (containing for example sulphur and phosphorus) the iron and a great part of the vanadium content of titanium-iron ores and the like. The process may also, so to speak, be carried 80 out in a fractional manner, insofar as at first only certain constituents are transformed into the sulphide phase by the sparing apportioning of the CaS added, and other constituents are thereupon transformed into a new 85 sulphide phase by the addition of CaS, MgS or Al<sub>2</sub>S<sub>3</sub>.

Naturally, not only heavy metals, but also light metals can be fractionally transformed in this manner from silicate or oxide into sulphide, for example, potassium, sodium and barium. If the process is carried out with these metals in the same manner as described above with reference to heavy metals care must be taken to ensure the simultaneous 90 presence of a sufficiently large heavy metal sulphide phase which is capable of taking up the freshly formed light metal sulphide, since the light metal sulphide would otherwise dissolve in the silicate slags, particularly when 95 the slag is basic. FeS is particularly suitable as a solvent for alkali metal sulphides. However in the production of these light metal sulphides a separation of the silicate phase and sulphide phase can be entirely disregarded, since these light metal sulphides are all water soluble and can therefore be subsequently extracted as a solution from solidified and disintegrated melt by lixiviation 100 with water. In this case it is moreover unnecessary to heat the mass to complete fusion, 105 since a moderate heating up to sintering and transformation is sufficient.

110 *Example No. 4.*—A prepared leucite from Italy contained 18% K<sub>2</sub>O, 2% Na<sub>2</sub>O, 23%, AlO<sub>2</sub>O<sub>3</sub>, 57% SiO<sub>2</sub>, it was finely disintegrated 115 together with 35% of gypsum and 7% of coke and was heated to sintering in a closed furnace, the gypsum being reduced to CaS which again reacted with the potassium content of the leucite. After cooling and disintegrating it was possible to lixiviate from the melt with water not only the potassium sulphide formed but also a large part of the 120 Al<sub>2</sub>O<sub>3</sub> content of the leucite which entered 125 into solution as potassium aluminate. From this solution the Al<sub>2</sub>O<sub>3</sub> can be obtained in known manner.

130 On the further addition of a certain amount of CaO to combine with the silicic

acid during the sintering process, the yield of potash and alumina is increased.

If already formed CaS is employed for reaction with leucite instead of gypsum and coke, the result is obtained that the transformation takes place at a much lower temperature, for example at 300° to 400° C. This result can be obtained by way of example, at a still lower temperature with the aid of an aqueous solution of CaS if a suitable moistened mixture is heated for a longer period with or without the employment of pressure. This process possesses the great advantage over the known process for the utilization of leucite by heating with CaO that CaS has a stronger tendency to react with silicate than CaO whereas on the other hand the freshly formed K<sub>2</sub>S has not such a strong tendency as K<sub>2</sub>O to be converted into the form of silicate.

As has been previously explained, it is possible, by means of the present process, in contradistinction to the former metallurgy, to obtain a clean cut separation in the liquid melt between sulphide (matte) and pure metal, by increasing the average heat of formation of the matte per gram-atom S up to 28 to 35 calories or more by the introduction of light metal sulphide. By employing this principle in the decomposition of mattes of diverse composition, the inventor has been enabled to obtain a better survey of the serial order of decomposition of metal from sulphide, i. e. over the partition of the different metals between sulphide and metal, than has been hitherto made available by metallurgy. Moreover the very important fact has been disclosed that the metallurgical speisses are in actual fact crude metals and not as has been hitherto assumed, matte-like products in which sulphur is replaced by arsenic (compare Ullman, Encyclopedie Techn. Chemie, vol. 7, pages 423 and 428). Whereas hitherto mattes and speisses have been tapped off together as a solution of liquid melts which only separated out into two layers in the tapping receiver on cooling, the method of conducting the smelting operation according to the present process however, yielded a clean-cut separation between matte and speiss even in the fused condition so that they could be separated from one another by tapping. Moreover numerous comparative tests demonstrated that the speisses according to their composition occupy a definite position in the serial order of precipitation of metal from the sulphide phase. This knowledge, in conjunction with the serial order of precipitation, established by the inventor, i. e. the partition of the different metals between metal layer and sulphide layer, enables the amount and composition of the speiss obtained to be regulated and moreover discloses a novel and economical method of working up speiss of valueless composition such as is frequently obtained in present day metallurgy.

The serial order of precipitation of the most customarily occurring heavy metals from a sulphide phase of the most diverse composition might be approximately the following Mo, As, Sb, Ag, Pb, Sn, (Zn above 1300°), Co, Ni, Fe, Cu, Cr, (Zn below 1200° C.), Mn. It is however, in this case, not a question of a well defined serial order, but of chemical equilibrium between metal phase and sulphide phase, which lead to the most diverse ratios of partition of the different metals between sulphide and metal, according to their position in the serial order of transference, their concentration in the system, and the degree of sulphidation of the system. By altering the latter the whole equilibrium can be displaced in one or other direction.

The serial order of precipitation is therefore in itself, insufficient as a basis of operation, inasmuch as for metallurgical operations the data relating to different definite states of equilibrium between metal phase and sulphide phase are necessary. For example, given a matte of the approximate composition 47% PbS, 12.9% Cu<sub>2</sub>S, 19.8% ZnS, 8.5% FeS, 0.84% As and about 10% (Na<sub>2</sub>S and CaS), which is subjected to decomposition by the removal of sulphur (for example by electrolysis), raw lead is first deposited until the lead content of the matte has been reduced to a definite quantity, which is interdependent upon the iron content of the matte. In the case of a higher iron content, if the lead content of the matte has been reduced to 10% to 8% Pb, both lead and iron are deposited in considerable quantity. The limiting values correspond to a lower lead content in the case of mattes with a poor iron content. From this stage onwards iron also separates out in addition to raw lead, which as is well known is not miscible with lead, and therefore appears as a definite metal layer above the lead. The following analysis taken from the experiments of the inventor show the partition of the different elements between matte and crude metal on smelting their raw materials at various adjusted degrees of sulphidation; incidentally Experiment No. 1 shows the case in which the sulphide phase has not separated off until metallic iron has appeared, and Experiment No. 2, shows the case in which the separation was continued until iron (-speiss) made its appearance.

#### Experiment No. 1

| Raw lead               | Matte                    | 125 |
|------------------------|--------------------------|-----|
| Pb not determined..... | PbS 15.27%               |     |
| Cu 1.98%               | Cu <sub>2</sub> S 22.70% |     |
| As 1.50%.....          | ZnS 35.20%               |     |
|                        | FeS 15.14%               |     |
|                        | As 0.18%                 |     |
|                        | Na <sub>2</sub> S 10.00% |     |
|                        | CaS                      | 133 |

## Experiment No. 2

|   | Matte                                                                                                   | Raw lead                                              | Speiss                                               |
|---|---------------------------------------------------------------------------------------------------------|-------------------------------------------------------|------------------------------------------------------|
| 5 | Pb 8.06%<br>Cu 15.20%<br>Zn 28.70%<br>Fe 14.20%<br>As 0.49%<br>Ag 80. gr. T.<br>Na <sub>2</sub> S 8.00% | As 0.56%<br>Ag 530 grams per ton<br>Pb not determined | As 24.7%<br>Cu 3.2%<br>Fe 63.3%<br>Pb not determined |

- 10 As can be seen from Experiment No. 1, the arsenic is distributed between matte and raw lead in the ration of about 1:8.2 as long as no iron separates out. During this period the raw lead is simultaneously speiss, as it were, inasmuch as it takes up arsenic. When however iron commences to separate out it thereupon extracts the bulk of the arsenic from the raw lead and from the matte and is converted into a speiss as can be seen
- 15 20 from Experiment No. 2. The partition ratio of the arsenic between iron, raw lead and matte shows a large preponderance in extraction by the iron, as can be seen. As is well known, iron is miscible to an extremely
- 25 slight extent with the ordinary non-ferrous metals such as lead and copper (and also tin) and forms a separate phase in the fused condition, side by side with these. Metals which in the simultaneous presence of iron
- 30 sulphide, metallic iron and non-ferrous metal, preferably collect in the iron phase, are advantageously classified as "siderophilic elements". Such siderophilic elements contain inter alia the following elements: Ni, Co,
- 35 Pt, Mo, As, Sb, P, C, Si. The mutual solubility of matte and speiss in the fused liquid state, known in present day metallurgical practice, is due to the fact the mattes hitherto contained practically no light metal sulphide and therefore possessed a high solvent power for pure metals, particularly for iron and siderophilic metals. The separation of such speisses from matte in the fore-hearth according to the hitherto usual practice is a
- 45 similar phenomenon to the known elutiation of metallic iron from its solution in FeS, by cooling. If no arsenic had been present in Experiment No. 2, crude metallic iron free from arsenic would have commenced to separate out as a separate phase at approximately the same temperature at which the iron speisses commenced to appear. For example, from a lead matte containing 5.85% Pb, 20.6% Fe, 28.9% Zn, and about 10% (Na<sub>2</sub>S + Ca) etc., a crude iron metal containing only 0.3% As was obtained together with crude lead. Experiment No. 2, shows that iron is an excellent collecting medium for arsenic and discloses the possibility of extracting the arsenic content from arsenical raw lead to a high degree, by the addition of some iron, and of recovering the same in a concentrated form.

50 The experiments moreover disclose the possibility of a new form of the old precipi-

tation process for lead, consisting in adding to the matte a certain amount of light metal sulphide, whereby the removal of lead from the matte to a lead-content of less than 8% can be effected. They further demonstrate the possibility of employing in this process iron speisses or copper speisses or copper-lead speisses instead of iron. In the latter case, it is possible by suitably adjusting the proportions, for example by the addition of an excess of speiss, to insure the production of small amounts of a fresh speiss of advantageous character, for example of iron speiss which acts as a collecting agent for the siderophilic elements present.

55 The two experiments also show the partition of the copper between the raw lead and matte (Experiment No. 1) and crude iron metal and matte (Experiment No. 2). From these and other experiments in the presence of large amounts of iron sulphide and metallic iron, a partition ratio of the copper between matte and crude metal is obtained, which lies between 1:10 and 1:6, generally however between 1:9.5 and 1.8. If for example no iron had been present in Experiment No. 2 the copper would have commenced to separate out when the matte had a lead content of about 1% Pb and would have extracted the arsenic from the raw lead and matte, forming copper speiss. Copper and lead are only miscible to a limited degree, but the presence of arsenic increases the miscibility, so that these copper speisses take up a considerable lead content from the raw lead simultaneously deposited. Such speisses are for example those which according to Ullman, Encyclopaedia Techn. Chemie, vol. 7, page 428, fall within the definition of ochre having a composition:

|       | Rich speiss | Poor speiss |
|-------|-------------|-------------|
| Cu    | 51.73       | 25.85       |
| Pb    | 35.20       | 16.68       |
| Fe    | 1.65        | 22.17       |
| As    | 2.75        | 4.04        |
| Sb    | 3.34        | 13.50       |
| Ni+Co | 0.37        | 2.71        |
| Zn    | 1.83        | 3.31        |
| Ag+Au | 0.175       | 0.095       |
| S     | 1.83        | 4.13        |

110 and which are at the present time worked up with difficulty in speiss furnaces. In view of the position of these speisses in the serial order of precipitation of metal from the sulphide phase according to the present process, it might be possible to obtain the precipitation of speisses of suitable composition, for example of iron speisses even during the smelting. These speisses may however be worked up as such with the greatest facility, by causing them to react with a matte containing light metal sulphide and PbS or FeS for example, in accordance with the pres-

70

75

80

85

90

95

100

105

110

115

120

125

130

ent process, the copper content reacting with  $\text{PbS}$  or  $\text{FeS}$  for example,



and forming matte, whereas the lead content of the speiss enters the freshly formed raw lead derived from the matte. The separated iron forms with the siderophilic elements As, Sb, Ni, Co, a fresh speiss with more advantageous properties. The noble metals mainly enter the raw lead whilst the zinc enters the matte.

The position of zinc in the serial order of reduction of metal from sulphide has not hitherto been correctly recognized since a position was ascribed to it between tin and lead. Zinc sulphide belongs to the non-metallic sulphides which are formed from their components, accompanied by a considerable heat of formation. Metallic zinc is capable of reducing the respective metal from "metallic" heavy metal sulphides to a considerable extent, if the temperature be maintained sufficiently low. At high temperature however, the volatility of the zinc becomes apparent since at such temperatures it is set free by the same metals which it was capable of reducing from their sulphides at lower temperatures. Thus for example in the important reaction:



is a reversible reaction which at lower temperatures proceeds from right to left to a great extent but which obeys the law of mass action. Accordingly

$$\frac{[\text{ZnS}] \times [\text{Fe}]}{[\text{FeS}] \times [\text{Zn}]} = \text{constant.}$$

If now the temperature is maintained at such a high level that zinc distils off, the equilibrium is disturbed and the reaction can in this manner, at the high temperature, be caused to a large extent to proceed from left to right. In cases where the phases have a composition approximate to that set forth in Experiment No. 2 the critical temperature in this case lies between  $1250^\circ$  and  $1300^\circ$  assuming always that the sulphide layer is covered by a slag layer of about 7 cm. depth. Below  $1200$  to  $1250^\circ$  C. extremely little zinc volatilizes whereas above  $1300^\circ$  C. zinc volatilizes to a high degree. In Experiment No. 2, the temperature was accordingly maintained at about  $1200$  to  $1250^\circ$  C. in order to collect the zinc in the matte and this test showed that it is actually possible to collect the zinc in the matte as sulphide in the presence of metallic iron. The zinc content of the speiss in Experiment No. 2 was not determined but judging from experience of other tests might have amounted to about 1 to 2%. In another case the following distribution of the

zinc (and copper) between matte and raw metallic iron was found:

Matte... 23% Zn, 18.4% Cu.  
Raw metallic iron... 0.51% Zn, 1.59% Cu.

In the reduction of  $\text{ZnS}$  by means of copper at low temperatures slightly more zinc enters the metal, apparently because zinc possesses a certain affinity for metallic copper. A test in this case gave the following results:

Sulphide layer... 34.3%  $\text{ZnS}$  (= 23.3% Zn), 56.2%  $\text{Cu}_2\text{S}$ , about 8%  $\text{Na}_2\text{S}$ .  
Metal layer... 10-12% Zn, 89% Cu.

From the given determination of the position of zinc in the serial order of transference from sulphide to metal the new fact is thus apparent that on the one hand zinc can be collected as sulphide in the matte in the presence of metallic iron at temperatures below about  $1250^\circ$  C. At temperatures above  $1250^\circ$  C., on the other hand, metallic zinc is liberated by the action of iron and other heavy metals.

Experiment No. 2 also shows the partition of the silver between matte and raw lead at a low silver content. The partition ratio is about 1:7. In another experiment with pyrites rich in silver three products were obtained, namely:

1. Matte with 2.9% Ag.
2. Crude metallic iron with 0.09% Ag.
3. Crude silver with 72.4% Ag and 24.6% Pb.

The partition of the nickel between a matte rich in iron sulphide and raw metallic iron can be seen from the following equilibrium mass obtained by experiment:

Matte... 44.6% Fe, 4.14% Ni, 14.5% Cu, 10% ( $\text{Na}_2\text{S} + \text{CaS}$ ).  
Iron... 82% Fe, 17.1% Ni, 2.5% Cu.

The partition ratio is thus about 1:4 and shows that relatively high percentage ferro-nickels or nickel-steels low in copper can be fractionally separated directly from natural magnetic nickel pyrites concentrates containing about 2 to 6% of nickel and 1 to 4% of Cu with the aid of the present process.

The partition ratio of molybdenum between iron sulphide and metallic iron is still more favourable for such direct production of ferrous alloys. A test showed:

Matte... 89%  $\text{FeS}$ , 2% Cu, trace of Mo, 10% ( $\text{Na}_2\text{S} + \text{CaS}$ ).  
Metal... 70% Fe, 0.12% Cu, 29% Mo.

In another case ferro molybdenum containing 58% Mo was separated out from a matte which contained only 0.3% Mo. During this operation the silicate phase simultaneously present contained only 0.05% Mo.

The above explanation should be sufficient to clear up the serial order of precipitation of the most commonly occurring metals from sulphide and with the aid of the smelting principle it is easily possible by suitable experiments also to arrange the rare metals in the series. As regards the position of the speisses as raw metals, which absorb arsenic

and antimony in this serial order of precipitation, it has been established that in this connection there are three main classes of speisses which appear in sequence during the continued splitting up of a complex lead, copper, iron matte, namely:

1. Raw lead containing As and Sb (lead speiss),
  2. Iron speiss or crude metallic iron,
  3. Copper speiss or copper-lead speiss.
- Iron speiss appears to possess the most favourable metallurgical properties amongst these, because on the one hand, it only takes up extremely small amounts of lead and copper and on the other hand because it attracts in addition to arsenic other siderophilic elements such as for example, Ni, Co, Mo, Pt etc., to a high degree. In certain circumstances it may also be advantageous to bring one and the same matte or raw lead into contact with poor speisses in sequence, that is to say, with raw metallic ferrous metals for the more complete extraction of the siderophilic elements. The counter-current principle can be advantageously employed however, in this case. Moreover in such case, the composition of the iron employed for the speiss formation plays a certain part inasmuch as if the speiss formed contains carbon, it separates more sharply from the non-ferrous metals than speiss poor in carbon. Raw metallic iron containing carbon is however, a better collector for certain carbide-forming siderophilic elements such as for example vanadium, molybdenum, chromium, etc. than that poor in carbon and has moreover the advantage of a lower melting point than said latter. In certain circumstances, phosphorous may also be employed with advantage as the means for lowering the melting point. Instead of effecting the speiss formation by direct reduction, during the first smelting, it can also be effected by the direct addition of for example, raw iron. Moreover for the extraction of certain elements from slags, a treatment of these alone with raw ferrous metal, may be advantageous, thus for example a large part of the vanadium content can be thereby recovered from the smelting of Mansfeld copper schist by bringing said latter in a fused condition in contact with iron whilst simultaneously increasing the degree of reduction of the slags.
- In general, the new state of knowledge above referred to, which is essentially based on the fact that a clean separation between the matte and the raw metals is attained by the light metal sulphide content of the matte, permits of operation to a far greater extent than has hitherto been possible with the polyphase system, slag, matte, raw ferrous metal and non-ferrous metal. Besides being capable of application to the non-ferrous metals (for example Pb, Cu, Sn) where apart from these latter, raw ferrous metal is also en-

countered, the present process may advantageously be applied to such ores in which besides slags and matte only raw ferrous metals or ferrous alloys are encountered inasmuch as in this case, (in contradistinction to the hitherto known metallurgy of iron), the three phase system, slag, matte, raw ferrous metal is utilized in order that certain constituents of the ore may collect in the matte whilst others, collect in the raw ferrous metal and others again collect in the slag. The process is naturally most suitable for raw materials containing sulphide, for example, sulphide ores such as magnetic nickel pyrites, molybdenum glance, and the like, incompletely roasted sulphide ores or oxide ores having a high sulphur content or complex iron ores, inasmuch as fractional precipitation of the metals in the presence of a sulphide phase effects an advantageous division. A very important advantage of the process resides in the fact that in the case of materials very rich in sulphur or raw metals, the light metal sulphide phase of the system can exert a desulphurizing action upon the raw metal by taking up metallic sulphide. Thus for example, iron can be desulphurized even down to the extent of 0.3% S by contact with an iron sulphide phase containing light metal sulphide. This desulphurization need not necessarily be carried out during the first smelting operation, but it may also be effected by subsequent treatment of the iron which contains sulphur, in a foil hearth in a three phase system according to the present process; light metal sulphide being added during this subsequent treatment. It is also simultaneously possible by means of this after treatment if desired, to convert the iron into special iron alloys, by the addition of sulphidic raw materials, for example  $MoS_2$ , magnetic pyrites containing nickel etc. The iron purified from this process still contains 0.3% S or more and must further be desulphurized in a subsequent operation according to known processes for example, by thermoelectrolysis. Whereas the object of the present day metallurgy of iron is to effect an intensive desulphurization during the first smelting operation by means of basic slags and intensive reduction and thus driving off the phosphorus content in the ore to a large extent into the iron, in the present process, on the other hand, no attention need be paid to the desulphurization in the first smelting operation but a high degree of dephosphorization can already be obtained if desired, in the first smelting operation by the low degree of reduction of the slags (low consumption of coke). If desired, the operation may also be conducted to produce directly iron with a low carbon content. Raw iron comparatively free from manganese can be obtained from impure iron ores containing sulphur with a low manganese content inasmuch as the man-

ganese content collects in the desired and suitably adjusted concentration in the sulphide phase and can subsequently be recovered, entirely free from phosphorus, from the latter in a known manner. This sulphidic manganese material can be converted into high grade oxidic manganese material by subsequently roasting and sintering. Impure chromium ores can be treated in a similar manner, since chromium also collects in the matte to a large extent. The extent of the metal phase, sulphide phase, slag phase, as well as the composition of the phases, can be regulated in this case by the composition of the charge, the amount of the added reducing carbon and the operation of the furnace according to known principles.

A further very important field of application of the process in the iron industry is that of a complementary operation to such known processes for working up sulphidic iron ores for which per se no practical use could be found owing to the fact that they yield a raw iron too rich in sulphur with the means hitherto available in practice. By subsequently treating such ores in a three phase system according to the present process, iron sulphide can be removed from iron thus produced, up to a remainder of 0.3% S. An important instance is the reduction of iron oxide by means of iron sulphide according to the well known reactions:



By this means iron with a low carbon content and concentrated  $\text{SO}_2$  are obtained. It is proposed in a Norwegian specification to cause pure oxidic iron ore (free from gangue) to react with pure iron sulphide for the purpose of producing iron. The reason for which this proposal has not been carried into practical effect may probably be due to the fact that even when using pure starting materials, the aforesaid reactions do not proceed sufficiently to completion at temperatures which are economical and practically available so as to produce iron, which is sufficiently free from S. According to the degree of the temperature employed, a sulphur content of 2 to 10% remains behind in the iron, the removal of which with the means hitherto available is too expensive. By combining this process with the present invention a relative independence of the degree of desulphurization in the first process is attained, since by subsequent treatment of the resulting iron which contains sulphur, in a three phase system with a sulphide phase containing light metal, the result is achieved of decreasing the content of iron sulphide in the iron to about 0.5%. Since in this embodiment, a very high degree of desulphurization is not necessary in the first operation, low temperatures are sufficient and the ores can advantageously be

employed with their usual content of gangue. This embodiment has the further great advantage over the direct desulphurization in one operation that a fractional precipitation of metal from sulphide is incidentally attained at the same time. If a low copper content is present as for example in Norwegian pyrites and burnt pyrites, this collects mainly in the sulphide phase during the second operation. This fractional recovery is still more important in the case of other more complex material and in such case the slag can also be utilized for the fractional collection of certain components. Taking into account the previous explanation, the possibilities in this connection can be immediately seen from the following equations:



Another known process which leads to the production of iron containing sulphur in a similar manner is the direct thermal decomposition of  $\text{FeS}$  into iron and sulphur.  $\text{FeS}$  is stable up to about  $1700^\circ \text{C}$ , and at increasing temperatures gives off increasing amounts of sulphur so that solutions of  $\text{FeS}$  in Fe of different composition are produced, according to the temperatures employed. These can be divided into sulphide phase and metal phase in exactly the same manner as explained with reference to the preceding process and either in the same apparatus (simultaneously) or one after the other. Elementary sulphur is obtained as a by-product. This process may also be combined with the preceding one if desired, and both S and  $\text{SO}_2$  may be produced. 95

The process may be carried into practical effect in any known metallurgical furnace, the aim however being to alter the operation of the furnace and the course of the process without making many alterations in the apparatus. Both shaft furnaces, reverberatory furnaces and electrical furnaces may be employed with advantage the apparatus being in each case selected to suit the particular purpose. It should however be remarked that electric fusion is particularly suitable for this purpose, and in particular, electrode furnaces with a deep slag bath as resistance with or without an arc between the slag bath and the electrodes, since such an arrangement furnishes the maximum temperature in the slag where it is most desired and can best be sustained. Such an arrangement is particularly advantageous in cases where, with a view to collecting zinc in the matte, it is necessary that the temperature thereof 100 115 120 125 130

should not exceed 1250° C. Even in cases where the process is carried out in shaft furnaces or reverberatory furnaces, electric furnaces can be employed as fore-hearths of the type which have an extremely favourable influence on the partition of the metal between the phases and are practically indispensable in cases where the different phases, either together or each separately, are intended to be subjected to a treatment with different raw ferrous metals. As a matter of fact it has been found that in a three phase system where it is intended to divide up a fused liquid solution of metal and sulphide into two phases by the addition of light metal sulphide, this division is effected more rapidly and cleanly if this system is subjected to the electrolytic action of an electric current.

I claim:-

20. 1. A process for smelting ores and other metallurgical products which comprises producing a polyphase system including the phases slag, matte and metal by a reduction smelting in the presence of light metal compounds, the amount of light metal compounds and the extent of reduction being so regulated as to produce a slag having an iron content of below 15% of FeO and a matte containing light metals.
25. 2. A process for smelting ores and other metallurgical products which comprises producing a polyphase system including the phases slag, matte and metal by a reduction smelting in the presence of light metal compounds, the amount of light metal compounds and the extent of reduction being so regulated as to produce a slag having an iron content of below 6% of FeO and a matte containing light metals.
30. 3. A process for smelting ores and other metallurgical products which comprises producing a polyphase system including the phases slag, matte and metal by a reduction smelting in the presence of light metal compounds including alkali metal compounds, the amount of light metal compounds and the extent of reduction being so regulated as to produce a slag having an iron content of below 15% of FeO and a matte containing light metals.
35. 4. A process as defined in claim 1 wherein heavy metal oxides are converted into sulfides and transferred to the matte phase by interaction with a sulfide of at least one of the metals, calcium and magnesium.
40. 5. A process as defined in claim 1 wherein heavy metal oxides are converted into sulfides and transferred to the matte phase by interaction with a sulfide of at least one of the metals, calcium and magnesium, the sulfides of calcium and magnesium being produced in situ during the process.
45. 6. A process as defined in claim 1 wherein heavy metal oxides are converted into sulfides and transferred to the matte phase by

interaction with a sulfide of at least one of the metals, calcium and magnesium, the sulfides of calcium and magnesium being produced in situ during the process by the interaction of carbonaceous material with the corresponding sulfates. 70

7. A process as defined in claim 1 wherein the charge and reduction is regulated to produce an acid slag.

8. A process as defined in claim 1 wherein the charge and reduction is regulated to produce an acid slag containing over 40% of silica. 75

9. A process as defined in claim 1 wherein such an amount of iron is provided in the charge that a metallic iron phase is produced for the absorption of siderophilic elements. 80

10. A process as defined in claim 1 wherein such an amount of iron is provided in the charge that a metallic iron phase is produced for the absorption of siderophilic elements and the reduction is so carried out that metalloids of the group consisting of carbon, silicon and phosphorus are present in the iron phase. 85

11. A process as defined in claim 1 wherein such an amount of iron is provided in the charge that a metallic iron phase is produced for the absorption of siderophilic elements and substantially non-ferrous speisses of metals non-miscible with iron are added to the charge whereby the metals non-miscible with iron contained in the non-ferrous speisses are liberated by interaction with the iron and production of an iron speiss. 90

12. A process for smelting ore and other metallurgical products which comprises producing a polyphase system including the phases slag, matte and metal by a reduction smelting in the presence of compounds of metals whose sulfides have heats of formation of over 40 kg. cal. per gram atom of sulfur, the amount of said metal compounds and the extent of reduction being so regulated as to produce a slag having an iron content of below 15% of FeO and a matte containing the sulfides of said metals. 100

In testimony whereof I affix my signature.  
HARALD SKAPPEL.

115

120

125

130

**Certificate of Correction**

Patent No. 1,797,700.

Granted March 24, 1934, to

**HARALD SKAPPEL**

It is hereby certified that error appears in the printed specification of the above-numbered patent requiring correction as follows: Page 7, line 70, for the character "MGCO<sub>3</sub>" read *MgCO<sub>3</sub>* and line 124, for "Na<sub>2</sub>" read *Na<sub>2</sub>S*; page 8, line 48, for "Al<sub>2</sub>O<sup>3</sup>" read *Al<sub>2</sub>O<sub>3</sub>* and line 116, for "AlO<sub>2</sub>O<sub>3</sub>" read *Al<sub>2</sub>O<sub>3</sub>*; page 10, line 90, for "1.8" read *1:8*; page 11, line 103, for "Fe, 17.1%" read *Fe, 17.15%*; page 13, line 89, in Equation 13, for "2Sn" read *Sn+2*; and that the said Letters Patent should be read with these corrections therein that the same may conform to the record of the case in the Patent Office.

Signed and sealed this 5th day of May, A. D. 1931.

[SEAL.]

**M. J. MOORE,**  
*Acting Commissioner of Patents.*